

Feb. 16, 1943.

W. T. HAGELIN

2,311,047

LITHOGRAPHIC PLATE AND PROCESS OF MAKING THE SAME

Filed Dec. 6, 1940



*Fig. 3*

Inventor:  
William T Hagelin  
By: Thies, Olsen & Macklen, bulger.  
Attys.

## UNITED STATES PATENT OFFICE

2,311,047

LITHOGRAPHIC PLATE AND PROCESS OF  
MAKING THE SAME

William T. Hagelin, Chicago, Ill.

Application December 6, 1940, Serial No. 368,753

15 Claims. (Cl. 41—41.5)

This invention relates to a lithographic plate and a process of making the same. More particularly, this invention relates to a process of producing a lithographic plate having a surface that is very receptive to greasy films such as may be applied thereto by crayon, lead pencil, grease ink, and the like or by a suitable stylus through a tracing sheet such as carbon paper or a typewriter ribbon.

A plate, to be useful in ordinary lithographic work, should be one that is treated in such a manner that the surface thereof is adapted readily to receive a grease coating or film such as may be made through a typewriter ribbon or by pencil, crayon, or other drawing or tracing instrument that is capable of depositing a greasy film on said surface when contacted therewith. The character of the surface should be such that after desired markings have been produced thereon, the portions of the surface not coated with the markings or grease film may be subjected to a treatment whereby those portions of the surface will be rendered ink-repellent while the coated portions remain very receptive to greasy substances such as lithographic ink. Consequently, when the lithographic plate having an image impressed thereon is passed under a roller containing a grease ink, the ink will adhere only to that portion of the plate to which the grease film or markings have been applied and a reproduction of the markings may be transferred directly to the surface to be printed or to a cylinder having a rubber blanket which in turn transfers it to the desired surface in accordance with the common practice. It is therefore important in the lithographic art that lithographic plates have a surface which at one time is strongly receptive to markings which may be produced by greasy materials, but which surface is also of such a character that it may be treated to render it grease-repellent except in those portions of the surface to which the greasy film or markings have been applied.

It is an object of this invention to provide an improved lithographic plate which is capable of readily receiving a greasy film from any sort of a drawing instrument, stylus or stencil capable of depositing on said surface a grease-containing film in selected areas.

A further object of this invention is to provide a continuous process of preparing a lithographic plate having the above indicated desirable characteristics.

A further object of this invention is the provision of a flexible lithographic plate and a

method of producing the same upon which a very ink-receptive image may be impressed either by means of direct contact or by means of photolithographic processes.

5 A further object of this invention is the provision of a metal surface coating which is substantially non-oxidizable even though exposed to the atmosphere under conditions normally promoting oxidation.

10 A still further object of this invention is the provision of a new etch solution which may be used for the treatment of lithographic plates.

Further additional objects will appear from the following description, the accompanying drawing, and the appended claims.

15 In accordance with one embodiment of this invention, a lithographic plate may be prepared from a metal sheet by subjecting one surface of the sheet to a graining treatment, and then subjecting said surface to the action of an alkali earth metal oxide and silica in the presence of water. These compounds apparently react with the metallic surface of the lithographic plate to form a deposit or coating which is extremely receptive to markings which may be impressed thereon by a grease-containing stylus such as a crayon or lead pencil, or which may be impressed thereon through ordinary carbon paper or a typewriter ribbon. The deposit renders the 20 surface of the metal treated very resistant to oxidation and the treated plates may be stored for long periods of time.

25 The process of producing lithographic plates of this invention may be continuous. In accordance with one embodiment of this invention, a continuous thin metal strip is passed under a revolving wire brush in order to remove foreign material from one surface of the strip, and to impart a desired grain thereto. The resulting 30 strip is then subjected to a scrubbing or brushing action in the presence of substantial quantities of a mixture of lime, finely divided silica, and water. During this scrubbing action a deposit or coating forms on the surface of the

35 metal sheet which is subsequently brushed and washed with water and thoroughly dried. The deposit or coating survives the subsequent washing and drying operations and is of such a nature that the surface of the resulting metal is very 40 receptive to grease markings imparted by contact or to other images produced in accordance with well known photolithographic processes.

45 The thus treated metal sheet may then be marked, scored, cut and packaged as desired.

50 It will, of course, be recognized that any type

of metal plate ordinarily used for lithographic work may be employed in carrying out this invention. While I prefer to use aluminum or zinc, it is within the scope of this invention also to employ stainless steel, Monel metal, or other metals or alloys which have been used in the lithographic art. If desired, a thin metal sheet may be employed which has a paper backing adhesively secured thereto. This paper backing is preferably waterproofed and secured to the sheet metal with a waterproof adhesive, so that subsequent contact of the resulting plate with water during treatment and during use will not cause separation of the paper and metal sheet. Also, while it is preferred to employ a mixture of water, lime and finely divided silica as the treating agent for the plate to form the desired grease-receptive deposit, it has been found that other alkali earth metal oxides may be substituted for the lime. Suitable substitutes are the oxides of barium, magnesium, and strontium. Under certain conditions, various silica-containing abrasives may be substituted for the silica, or other finely divided abrasives may be used, such as pumice, finely divided argillaceous materials and the like. However, I prefer to use finely divided silica of a fineness sufficient to pass a 250 mesh screen. It is the combination of the alkali earth metal oxide with silica and water which appears to produce the desired coating or deposit. Under certain conditions, a water-soluble blue dye may be incorporated with the treating mixture in order to impart a desirable whiteness to the coating on the resulting plate. Only traces of the blue dye may be used, a suitable one being a water-soluble dye known as benzoyl blue.

For a more complete understanding of this invention, reference will now be had to the drawing, wherein Figure 1 is a diagrammatic elevational view of an apparatus which may be used for a continuous process of producing a lithographic plate in accordance with one embodiment of this invention.

Fig. 2 is a greatly enlarged partial sectional view of a lithographic plate prepared in accordance with one embodiment of this invention, having the coating or deposit of ink-receptive material thereon.

Fig. 3 is similar to Fig. 2, but shows a product having a backing of waterproofed paper adhesively secured to the sheet.

Referring now more particularly to Fig. 1, a roll 10 of thin sheet metal is provided which is capable of being unrolled to advance a continuous strip of metal 12 over a table 14 of Monel metal, glass, or other corrosion-resistant material, by means of drawing rolls 16. The sheet 12 may be a thin metal sheet of aluminum or zinc or other lithographic metal having a thickness of about  $\frac{1}{1000}$  inch. Such a sheet is flexible and is, when treated, capable of being inserted into the carriage of an ordinary typewriter and positioned on the drum of an ordinary lithographic machine. If desired, the metal sheet 12 may be provided with a paper backing 18, as indicated in Fig. 3. In such case, the metal sheet may have a thickness of about  $\frac{1}{1000}$  inch, and the backing a thickness of about  $\frac{1}{1000}$  inch. The backing is preferably waterproof paper, and adhered to the metal sheet 12 by means of a waterproof adhesive. It will be understood, of course, that the metal sheet or the metal sheet and paper backing may be of any desired thickness and I do not wish to limit myself to the particular

dimensions indicated above. The metal surface of the strip 12 has been, prior to the time that it is rolled into the roll 10, treated with a wire brush, in order to remove foreign matter from the surface of the metal and to provide a suitable roughness or grain to the surface of the strip to be treated.

The strip 12 having the grained surface is pulled continuously from the roll 10 by means of the drawing rollers 16 under a spout 20 of a receptacle 22 having contained therein a mixture 24, which is deposited on said strip. The mixture 24 preferably comprises about two parts by weight of calcium oxide, about two parts by weight of finely divided silica, and about eight parts by weight of water. A small amount of benzoyl blue may also be added thereto in order to provide a desired whiteness to the coated surface of the resulting product. The mixture 24 within the receptacle 22 is continuously stirred by a paddle 26 operated by means (not shown) through a belt 28. By this means, the ingredients in the mixture 24 are kept in uniform suspension and undesirable settling is prevented. The mixture 24 is deposited through the spout 20 onto the grained surface of the metal sheet 12 which is continuously advanced under a doctor blade 30 serving evenly to distribute the mixture over the entire surface of the sheet. The thus covered sheet is then passed over the table 14 and under a plurality of oppositely rotating brushes 32 which serve to scrub the surfaces of the sheet in the presence of the mixture of lime, silica, and water, and to thoroughly contact the mixture with the grained surface of the sheet. The sheet 12 is then advanced under a squeegee 34 in order to remove excess quantities of the mixture, and then is advanced under a plurality of washing brushes 36 which also rotate in opposite directions and serve to remove all traces of excess quantities of silica and lime from the surface of the sheet. Water for the washing brushes 36 is sprayed on the brushes through a plurality of pipes 38 positioned thereabove. The corrosion-resistant table 14 serves as a backing for the scrubbing brushes 32 and the washing brushes 36.

The strip 12, after having been washed, is then passed under a cloth-covered wiping roll 39 and between the drawing rolls 16, which latter serve to pull the sheet 12 across the table 14, and which also serve to squeeze excess quantities of water from the sheet 12, in case such sheet has a paper backing, as indicated in Fig. 3. The sheet 12 is then advanced through a drying chamber 40, which is equipped with a plurality of drying lights 42 positioned above and below the sheets. The product here may be re-rolled if desired and may be subsequently marked, cut and packaged as needed. However, as shown in the drawing, it is fed directly from the drying chamber 40 into a printing mechanism 44, which prints, with water color ink, markings to serve as guide marks on the resulting product, and thereafter it is fed into a scoring device 46, and to the cutters 48, which serve to cut the sheet to the desired lengths. The separate sheets may then be stacked and packaged in any desired manner.

It will, of course, be recognized that both surfaces of the strip 12 may be treated in accordance with this invention. It is, in such a case, necessary to subject both sides to a prior wire brushing or graining operation before treating the product as herein disclosed. This double treatment may be applied to both sides of a

metal sheet or to the exposed surfaces of two metal sheets adhered to each side of a water-proofed paper backing by a waterproof adhesive.

It has been discovered that a lithographic plate prepared in accordance with the process indicated above has many desirable properties which make it superior to lithographic plates which have heretofore been used in the art. It is very receptive to grease, and is consequently very useful for accurately reproducing grease markings which may be impressed thereupon. After desired markings have been impressed on the plate, either mechanically by a typewriter or other drawing instrument or by a photolithographic operation, the surface of the plate may be wiped with a sponge containing a solution which is known in the lithographic art as an etch solution whereby those portions of the surface not containing the greasy material or photographic image are rendered ink-repellent. A particularly useful etch solution prepared in accordance with this invention has the following composition:

|                         |                                                   |      |
|-------------------------|---------------------------------------------------|------|
| Distilled water         | ounces                                            | 32.0 |
| Glycerine (Y. D.)       | do                                                | 4.4  |
| Mono-ammonium phosphate | grams                                             | 28.8 |
| Ammonium sulfate        | do                                                | 2.0  |
| Phosphoric acid         | Sufficient to adjust the solution to about pH 3.8 |      |

This etch has properties which make it superior to other etches of which I am aware.

After the plate has been treated with the etch solution, it may be mounted on the drum of a lithograph machine and a grease ink may be applied to the surface of the plate by means of a roll. The ink will adhere only to those portions to which the grease film or markings have been applied and the grease ink on these markings may then be transferred directly to the surface to be printed or to a cylinder having a rubber blanket which in turn transfers it to the surface to be printed. A fountain etch may be applied to the plate by means of a water roll on the lithograph machine in order to insure that the ink-repellent portions of the plate will retain their ink-repelling properties. In accordance with one embodiment of this invention, a suitable fountain etch is one which may be prepared by adding an equal quantity of glycerine (Y. D.) to the etch composition given above.

Plates prepared in accordance with this invention retain their accuracy of reproduction over long periods of time and may be used indefinitely. They are also very resistant to oxidation and the plates may be stored for long periods of time and re-used. This non-oxidizing coating imparted to the surface of the metal in accordance with this invention may be applied to other metal articles such as they be employed in structural work but, of course, it finds particular use in the preparation of lithographic plates as herein described.

An important feature of the present invention is the provision of a lithographic plate which has been treated with a mixture of water, an alkali earth metal oxide and silica. Any desired proportions may be used but I have discovered that best results are obtainable when about equal parts of the oxide and silica are used in admixture with a somewhat greater amount of water. This mixture when applied as indicated above forms a deposit or coating on

the surface of the lithographic plate. This coating is indicated at 50 in Figs. 2 and 3. I do not understand what the true nature of this coating is, nor do I understand the nature of any physical or chemical reactions that may be involved in its formation. However, I do know that the use of the mixture indicated results in an improved lithographic plate which is much more receptive to grease images than are plates which have been prepared and cleaned with ordinary abrasives or chemical cleaning agents.

The plate of this invention is extremely fine-grained and is capable of transferring an extremely accurate image. Markings of lead pencil, crayon and grease ink on the plate are accurately reproducible and are readily distinguishable one from the others on the surface printed with the plate of this invention. The markings on the plate can be erased in case corrections are desired while the markings are being applied thereto. Erasures may be made by a stiff glass fiber brush or by means of a suitable solvent, such as a mixture of equal parts of trichlorethylene and acetic acid. The erasures are indistinguishable in the reproduction and fresh markings may be applied to the plate over the erasures.

While particular embodiments of this invention are shown above, it will be understood, of course, that the invention is not to be limited thereto, since many modifications may be made, and it is contemplated, therefore, by the appended claims, to cover any such modifications as fall within the true spirit and scope of this invention.

I claim:

1. A process of preparing a lithographic plate which comprises imparting a grain to one surface of a metal sheet, treating said surface with a mixture of an alkali earth metal oxide, silica and water, washing said mixture therefrom, and drying the resulting product, whereby said surface has been rendered strongly receptive to impressed greasy markings.
2. A process of preparing a lithographic plate which comprises imparting a grain to one surface of said plate, scrubbing said surface in the presence of a mixture of lime, finely divided silica and water, washing said mixture from said surface, and drying the plate, whereby said surface has been rendered strongly receptive to impressed greasy markings.
3. A process of treating the surface of a metal plate to render it strongly receptive to impressed greasy markings comprising imparting a grain to said surface, brushing said surface in the presence of a mixture of lime, finely divided silica and water, then washing said mixture from said plate, and drying the same.
4. A process of treating the surface of a metal plate to render it strongly receptive to impressed greasy markings comprising the steps of wire-brushing said surface to impart a grain thereto, depositing a mixture of lime, silica and water on said surface, brushing said surface in the presence of said mixture with a plurality of oppositely rotating brushes, washing and brushing said mixture from said surface, and drying the plate.
5. A process of treating the surface of a metal strip to render it strongly receptive to impressed greasy markings comprising imparting a grain to said surface, continuously advancing said strip, depositing a mixture of lime, silica and water on said surface, brushing said surface in the presence of said mixture with a plurality of oppositely rotating brushes, washing and brushing said mixture from said surface, and drying the plate.

ence of said mixture as the strip continuously is advanced, then washing said mixture from said surface, drying the same, and cutting the strip into predetermined lengths.

6. The process of claim 5 in which said strip is continuously marked and scored prior to cutting.

7. An etch solution for treating the surfaces of lithographic plates comprising water, glycerine, mono-ammonium phosphate, ammonium sulfate and phosphoric acid.

8. A process of preparing a lithographic plate which comprises treating the surface of said plate with a mixture of an alkaline earth metal oxide, finely divided silica and water whereby a grease receptive coating is formed thereon, applying desired grease markings to said surface, and treating said surface with an etch to render grease-repellent those portions of the surface not covered with the markings, said etch comprising an aqueous solution of glycerine, mono-ammonium phosphate, ammonium sulfate, and phosphoric acid, whereby to form a fine-grained plate capable of transferring an extremely accurate image of said grease markings.

9. A process of preparing a lithographic plate which comprises imparting a grain to one surface of a metal sheet, treating said surface with a

mixture of an alkali earth metal oxide, a finely divided abrasive and water, washing said mixture therefrom, and drying the resulting product, whereby said surface has been rendered strongly receptive to impressed greasy markings.

10. A lithographic plate comprising a thin flexible metal sheet having the normal lithographic surface thereof grained and treated with a mixture of an alkaline earth metal oxide, a finely divided abrasive, and water to provide a grease-receptive coating thereon.

11. The lithographic plate recited in claim 10 wherein said abrasive comprises silica.

12. The lithographic plate recited in claim 10 wherein said alkaline earth metal oxide comprises lime.

13. The lithographic plate recited in claim 10 wherein said sheet comprises aluminum.

14. The lithographic plate recited in claim 10 wherein a sheet of waterproofed paper backing is adhesively secured to the opposite surface of said metal sheet.

15. A lithographic plate comprising a thin flexible aluminum sheet having the normal lithographic surface thereof grained and abraded with a mixture of lime, finely divided silica, and water to provide a grease-receptive coating thereon.

WILLIAM T. HAGELIN.